

Aug. 9, 1932.

J. B. WELLS

1,870,662

COLOR BACKED MOTION PICTURE FILM

Filed May 17, 1930



Inventor,  
*Jackson B. Wells,*

By *Newton M. Perrius*

Attorney

## UNITED STATES PATENT OFFICE

JACKSON B. WELLS, OF ROCHESTER, NEW YORK, ASSIGNOR TO EASTMAN KODAK COMPANY, OF ROCHESTER, NEW YORK, A CORPORATION OF NEW YORK

## COLOR BACKED MOTION PICTURE FILM

Application filed May 17, 1930. Serial No. 453,341.

This invention relates to motion picture film, and particularly to the type of film which is backed with a dye which later bleaches out during processing.

In the case of amateur motion picture film particularly, where excessively contrasting lightings are sometimes encountered, it has been customary to some extent to back the film with a dye designed to eliminate halation. The dyes used bleach out on processing the film and disappear. In the case of the ordinary cellulose acetate support it is sometimes difficult to completely bleach out certain of the desirable dyes. This is, of course, 15 objectionable as a certain tint or over-all grayness remains over the image.

An object of this invention is to facilitate the bleaching out of colored backings put on for the purpose indicated.

20 The single figure of the accompanying drawing shows in perspective and cross-section an embodiment of my invention.

I have found that a thin backing of cellulose acetate of a definite description coated 25 on the regular cellulose acetate support, but under the color backing, permits the non-halation dye to bleach out more perfectly than an unbacked support.

The kind of cellulose acetate I employ for 30 this intermediate backing is one of relatively low precipitation value, and one which gives a clear solution containing a minimum amount of haze or insoluble particles of acetate when dissolved in acetone. I have 35 found that in making up these solutions these fine particles which are not soluble in acetone cannot be removed by filtration and therefore give trouble when cotton is used showing this haze. On the other hand, solutions 40 which show no haze are desirable for the application of the undercoat as I use it.

The term "precipitation value" is an arbitrary one and is defined in co-pending application Serial No. 353,649, filed by A. F. Sulzer, April 8, 1929. The term "precipitation value" is applied to the results of certain definite tests which are carried out in the following way. Five grams of the dry cellulose acetate are accurately weighed and placed in a wide-mouthed 12 ounce bottle. To this

are added 100 cc. of acetone (commercial grade of 99% or better), and the mixture is stirred until homogeneous. The bottle should be closed during the stirring with a rubber stopper fitted with a shaft for the stirrer. 55 To this dope is added slowly from a pipette and with thorough stirring 150 cc. of a mixture consisting of two parts of distilled water and one part of acetone by volume. Care should be taken to keep the solvent mixture 60 at 20° centigrade wherever volumes are being measured.

At the end of the addition of the acetone and water mixture, a mixture is obtained containing 40% water by volume (neglecting contraction) in which is suspended the precipitated acetate. This is allowed to stand for 12 hours at 20° centigrade. 25 cc. of the clearest portion (super-natant solution) are removed with a pipette. At the end of this 70 time precipitation has reached equilibrium and proceeds no further, and during the same time settling of the precipitate occurs. This 75 25 cc. is centrifuged in stoppered bottles at high speed until the liquid is perfectly clear. Exactly 5 cc. of the clear liquid are removed with a pipette and evaporated to dryness on a weighed watch glass. If W is the weight of the residue in grams, the precipitation 80 value which equals the per cent acetate precipitated,

$$= 100 - W \times \frac{250}{5} \times \frac{1}{5} \times 100 \\ = 100 - 1000W$$

The cellulose acetate which I use has preferably a precipitation value of about 70% when calculated in this manner. I may use, however, so far as the purposes of this invention are concerned, an acetate of precipitation value as low as 25%, or of any value between 25% and 75%. Such an acetate is more susceptible to water and bleach baths than cellulose acetate of higher precipitation value, the product of the latter type showing the property of higher resistance to water.

In carrying out my invention, all the processes may be performed continuously with the film forming operation. After the

main body of the support 3 is formed, preferably of a composition including cellulose acetate of high precipitation value, that is over 75% and preferably over 90%, I next apply to it a thin solution of approximately 2½% of cellulose acetate of the type specified, in acetone, for example. Other suitable solvents of course may be employed, but acetone is usually preferable. The operation of applying a thin coating of cellulose acetate is carried out on a coating machine of a well known type. This coating 4 dries very rapidly, and being very thin, its presence on the support can scarcely be detected. The intermediate coating of low precipitation acetate becomes integral with the support, there being no definite line of demarcation between the two, as indicated in the figure. The film is next passed through a machine which applies the color backing 5. For this purpose I use dyes of the general sort disclosed in the patent to Hickman No. 1,638,577, August 9, 1927. I of course do not limit myself to the particular dyes mentioned there and include broadly any dyes suitable for the purpose. It is also understood that any dye used in this manner must be capable of bleaching out or washing out in the subsequent processing of the film, that is, in the developer, the fixing bath, or the wash water.

The product as made by my invention may best be understood by reference to the drawing. A regular cellulose acetate support 3 has coated on it the intermediate backing 4 of acetate of low precipitation value. The outer face of the coating 4 carries the color backing or dye layer 5. The opposite side of the support carries the emulsion layer 2. As used for motion pictures the films has the regular perforations 1.

I have found that color backed film made in accordance with this invention bleaches out clearer than if the special acetate under-coating had not been used. The advantages of having a clear print after processing are readily apparent since such a print will give a cleaner picture on projection, will be better for sound reproduction, and will also require less light on exposure if other prints are made from it.

What I claim is:

1. A photographic film base comprising a support of cellulose acetate, an intermediate backing of cellulose acetate of low precipitation value and a color backing.
2. A photographic film base comprising a support of cellulose acetate, an intermediate backing of cellulose acetate of a precipitation value of the order of 70% and a color backing.
3. A photographic film base comprising a support of cellulose acetate, an intermediate backing of cellulose acetate of a precipitation value of the order of 70% and which

gives a clear solution with a minimum amount of haze in acetone, and a color backing.

4. A photographic film base comprising successively a support of cellulose acetate, an intermediate backing of cellulose acetate of low precipitation value and a superficial coating of a dye thereon.

5. A photographic film base comprising a support of cellulose acetate and an intermediate backing of cellulose acetate of low precipitation value having thereon a superficial coating of a dye which prevents halation.

6. A photographic film base comprising a support of cellulose acetate and an intermediate backing of cellulose acetate of low precipitation value having thereon a superficial coating of a dye which prevents halation and which bleaches out in the photographic processing baths.

7. A photographic film base comprising a support of cellulose acetate of high precipitation value and an intermediate backing of cellulose acetate of substantially lower precipitation value having thereon a superficial coating of a dye which prevents halation and which bleaches out in the photographic processing baths.

8. A photographic film base comprising a support of cellulose acetate and an intermediate backing of cellulose acetate of a precipitation value not over 75% having thereon a superficial coating of a dye which prevents halation and which bleaches out in the photographic processing baths.

Signed at Rochester, New York, this 12th day of May, 1930.

JACKSON B. WELLS.

105

110

115

120

125

130